

July 10, 1928.

1,676,709

M. POLANYI ET AL

## PROCESS FOR DETERMINING THE COMPOSITION OF COPPER AND ZINC ALLOYS

Filed Feb. 25, 1927



### Inventors:

Michael Polanyi  
Stephan von Orgas

Patented July 10, 1928.

1,676,709

# UNITED STATES PATENT OFFICE.

MICHAEL POLANYI, OF BERLIN-ZEHLENDORF MITTE, AND STEPHAN VON BOGDANDY,  
OF BERLIN-DAHLEM, GERMANY.

## PROCESS FOR DETERMINING THE COMPOSITION OF COPPER AND ZINC ALLOYS.

Application filed February 25, 1927, Serial No. 171,011, and in Germany March 24, 1926.

Our invention has for its object to provide a new process of determining the composition of copper and zinc alloys and especially of brass. The chemical analysis of brass or of alloys of copper and zinc in general, especially for the purpose of shop control during the course of manufacture and preparation, presents a number of difficulties, seeing that the determination of the 5 quantities by chemical means requires a great expenditure of time and pains as well as experience, and is further lacking in accuracy. When metallic copper and zinc are melted together for obtaining brass, 10 there is always a danger of the zinc oxidizing in the presence of air and accordingly escaping from the alloy. For this reason it is impossible to say beforehand what the exact composition of the alloy will be. In 15 this case it is absolutely impossible to apply chemical analysis, as during the melting process the time is too short to analyze the composition chemically and to make up possible losses of zinc by adding new metal.

20 By means of the present process these drawbacks are eliminated.

The process consists in heating the brass or other alloy to be examined in the form of drillings, powder, millings, grains and 25 the like in a vessel of quartz glass, glass with a very high fusing point, zircon, iron or the like in as high a vacuum as possible to such an extent that the zinc passes off by distillation, the copper and the like remaining 30 behind. By weighing the metal thus treated before and after heating to a point where no further changes of weight take place the amount of zinc present is determined.

35 In the accompanying drawing a device 40 suitable for this process is shown, by way of example, in diagrammatical manner.

*a* is a furnace, an electric furnace, for instance.

A vessel *c* which is almost cylindrical, or 45 preferably slightly tapered upwardly, is considerably reduced in diameter at *b*. This vessel is connected by means of metal, linings or sleeves *d* to a high vacuum tube *e*. The linings or sleeves *d* are preferably provided with a cooling system *f*, to allow cooling water to flow through. A weighing 50 glass *g* containing the metal to be examined is introduced by means of a hook, for instance, or the like into the reduced portion 55 *b* of the vessel *c*, and after connecting the

latter to the vacuum pipe *e*, heating takes place in the heater *a* until the weight remains constant. The heating is shown to be an electrical heating, the proper heating degree is adjusted by means of a resistance coil *a<sup>1</sup>* and an amperage indicator *a<sup>2</sup>*. The heater *a* is also connected to the cooling system by means of the pipes *h*, *h*. The vacuum required is produced by means of a mercury pump or the like, which is also 60 connected to the cooling system by means of pipes *k*, *k* and may also be connected by means of pipe *l*, to a device or system not especially shown and adapted to produce a prior degree of vacuum. Within tube *e* we 65 have provided a closing device such as cock *m*, an air entrance pipe *n*, and a vacuum measuring device *o* of any approved structure. The distilled zinc is condensed in that 70 part of the vessel *c* next the sleeve. A portion may also be condensed at a point higher 75 up, at *e*. Should it be desired to recover the zinc quantitatively and thus prove the correctness of the analysis, a plug of asbestos, glass or even wool or the like can be 80 introduced into the receptacle *c* at *c<sup>1</sup>*, after cooling, and after analysis weighing may be performed, or, after dissolving, a titration 85 or any other analytic means for determining may be restored to. The heating at *a* takes 90 place in accordance with the degree of volatility of the metal treated. As a rule a temperature is used ranging from 800° to 1100°.

In place of an electric heater *a* gas or 90 alcohol lamp or the like may also be used.

The vessel *g* may also be of quartz glass or other substance or metal of sufficiently refractory nature.

The possibility of zinc volatizing so 95 rapidly from alloys of copper and zinc is surprising. It could not be anticipated that such large quantities would escape within such a short space of time. On the contrary, it was not unreasonable to expect that 100 part of the metal would be retained. Our new method proved quite successful for all practical purposes.

What we claim as our invention and desire to secure by Letters Patent of the 105 United States, is:—

1. A process for determining the composition of alloys of copper and zinc, consisting in weighing a portion of the alloy to be treated, subjecting said weighed portion 110

to the action of heat in a vacuum until all the zinc contained in said alloy is volatilized, and weighing the remaining metal.

2. A process for determining the composition of alloys of copper and zinc, consisting in weighing a portion of the alloy to be treated, subjecting said portion to the action

of heat in a vacuum, maintaining said heat between 900° and 1100° until all the zinc contained in said alloy is volatilized, and 10 weighing the remaining metal.

MICHAEL POLANYI,  
STEPHAN yon BOGDANDY.